

# United States Patent [19]

Grenoble

[11] 3,905,842

[45] Sept. 16, 1975

[54] **METHOD OF PRODUCING SILICON-IRON SHEET MATERIAL WITH BORON ADDITION AND PRODUCT**

[75] Inventor: **Herbert E. Grenoble**, Amsterdam, N.Y.

[73] Assignee: **General Electric Company**, Schenectady, N.Y.

[22] Filed: **Sept. 23, 1974**

[21] Appl. No.: **508,330**

## Related U.S. Application Data

[63] Continuation-in-part of Ser. No. 431,128, Jan. 7, 1974, abandoned, which is a continuation-in-part of Ser. No. 326,852, Jan. 27, 1973, abandoned.

[52] **U.S. Cl.** ..... 148/111; 75/123 B; 75/123 L; 148/31.55; 148/112

[51] **Int. Cl.** ..... H01f 1/04

[58] **Field of Search** ..... 148/111, 110, 112, 31.55; 75/123 B, 123 L

[56]

## References Cited

### UNITED STATES PATENTS

|           |         |                    |         |
|-----------|---------|--------------------|---------|
| 3,575,739 | 4/1971  | Fiedler.....       | 148/111 |
| 3,700,506 | 10/1972 | Tanaka et al.....  | 148/111 |
| 3,725,143 | 4/1973  | Alworth et al..... | 148/112 |

### FOREIGN PATENTS OR APPLICATIONS

|         |        |            |         |
|---------|--------|------------|---------|
| 40-7663 | 4/1965 | Japan..... | 148/111 |
|---------|--------|------------|---------|

*Primary Examiner*—Walter R. Satterfield  
*Attorney, Agent, or Firm*—Charles T. Watts; Joseph T. Cohen; Jerome C. Squillaro

[57]

## ABSTRACT

The addition to silicon-iron of a small amount of boron in critical proportion to the nitrogen content of the metal enables preparation of oriented silicon-iron sheet of good magnetic properties from material which would otherwise be incapable of secondary recrystallization necessary to produce such properties.

**10 Claims, No Drawings**

## METHOD OF PRODUCING SILICON-IRON SHEET MATERIAL WITH BORON ADDITION AND PRODUCT

This is a continuation-in-part of my copending patent application Ser. No. 431,128, now abandoned, filed Jan. 7, 1974, which is a continuation-in-part of my patent application Ser. No. 326,852, filed Jan. 27, 1973 (now abandoned), both of which patent applications have been assigned to the assignee hereof.

The present invention relates generally to the art of producing electrical steel and is more particularly concerned with a novel method of producing singly oriented silicon-iron sheet through the use of small but critical amounts of boron, and with a new cold-rolled silicon-iron sheet product.

### CROSS-REFERENCES

This invention is related to the invention disclosed and claimed in patent application Ser. No. 429,800, now abandoned, filed Jan. 2, 1974 as a continuation-in-part of patent application Ser. No. 320,668, filed Jan. 2, 1973 (now abandoned), entitled "Method of Producing Oriented Silicon-Iron Sheet Material With Boron Addition" in the name of Howard C. Fiedler and assigned to the assignee hereof, directed to the novel concept of cold rolling hot-rolled silicon-iron sheet directly to final thickness without an intermediate heat treatment through the use of small but critical amounts of boron and by maintaining the ratio of manganese to sulfur in the metal at less than 1.5.

The invention disclosed and claimed herein also relates to that disclosed and claimed in patent application Ser. No. 429,791, now abandoned, filed Jan. 2, 1974, as a continuation-in-part of patent application Ser. No. 320,669, filed Jan. 2, 1973 (now abandoned), entitled "Method of Producing Oriented Silicon-Iron Sheet Material With Boron Addition" in the name of Howard C. Fiedler and assigned to the assignee hereof, which pertains to the new concept of using small but critical amounts of boron to enable the production of singly oriented silicon-iron sheet of improved magnetic properties by subjecting silicon-iron sheet containing manganese and sulfur in a ratio less than 2.1 to a cold reduction sequence including an intermediate annealing step and a final heavy cold rolling reduction.

### BACKGROUND OF THE INVENTION

The sheet materials to which this invention is directed are usually referred to in the art as "electrical" silicon steels or, more properly, silicon-irons and are ordinarily composed principally of iron alloyed with about 2.2 to 4.5 percent silicon and relatively minor amounts of various impurities and very small amounts of carbon. These products are of the "cube-on-edge" type, more than about 70 percent of their crystal structure being oriented in the (110)[001] texture, as described in Miller Indices terms.

Such grain-oriented silicon-iron sheet products are currently made commercially by the sequence of hot rolling, heat treating, cold rolling, heat treating, again cold rolling and then final heat treating to decarburize, desulfurize and recrystallize. Ingots are conventionally hot-worked into a strip or sheet-like configuration less than 0.150 inch in thickness, referred to as "hot-rolled band." The hot-rolled band is then cold rolled with appropriate intermediate annealing treatment to the fin-

ished sheet or strip thickness usually involving at least a 50 percent reduction in thickness, and given a final or texture-producing annealing treatment.

### SUMMARY OF THE INVENTION

I have discovered that under certain conditions boron has a beneficial effect on the secondary recrystallization of silicon-iron sheet material to develop the (110)[001] texture and the special magnetic properties associated with it. Particularly, I have found that the presence of a very small, but highly critical, amount of boron in cold-rolled silicon-iron sheet during the final or texture-developing anneal enables preparation of silicon-iron sheet having a strong cube-on-edge texture and correspondingly good magnetic properties. In other words, the seemingly insignificant amount of boron makes secondary recrystallization possible. Consequently, the use of manganese sulfide can be avoided as can the necessity of a high-temperature desulfurizing heat treatment during the final processing operations. Thus, the metal can by reason of this invention be desulfurized at the melt stage with substantial time and cost savings. All this is quite surprising, considering the fact that boron has previously been recognized in our experience as a detrimental impurity which it definitely is in amounts only moderately greater than those which I have found to be useful. In fact, except in the presence of otherwise detrimentally high amounts of nitrogen in the metal, boron in amount as small as 50 parts per million (ppm) is definitely detrimental in terms of desired magnetic characteristics. Thus, the important new results and advantages of this invention are obtained through the presence of boron in amounts from about five to about 45 ppm during the texture anneal of the cold-rolled sheet. I have found the optimum boron content to be in the range from about five to 20 ppm.

This unique capability of boron was discovered during experiments involving the use of crucible refractories containing boron as a minor impurity. Small amounts of boron were reduced from the refractories to the silicon-iron melts and exerted noticeable beneficial effect on the texture-developing process. Subsequently, I demonstrated that the boron content in silicon-iron melts prepared in such vessels could be closely controlled by adjusting the melt carbon content as by adding iron oxide and thereby preventing the reduction of boron in the crucible refractory and consequent pick-up of boron by the melt. I further found that the boron requirements can be met through the use of a boron-free crucible by adding a boron source to the melt.

I have further found that the surprisingly sharp criticality of such relatively small proportions presents no substantial difficulty in either laboratory or mill-scale operations. Thus, boron in suitable form is added in requisite amount to the melt shortly before casting. In mill practice, the boron source is suitably added to the ladle after the usual ferrosilicon addition. No significant loss of boron from the metal occurs through hot and cold rolling and heat treating stages prior to the final heat treatment. However, boron loss can be substantial if the boron source is added well in advance of casting or if the ingot is soaked at high temperature for a prolonged period. During the final anneal, essentially all the boron is eliminated from the metal when in accordance with this invention the role of boron in pro-

moting the desired secondary recrystallization texture development has terminated.

I have additionally discovered that the proportion of nitrogen to boron is also of critical importance to the new results and advantages of this invention. Unless the ratio of nitrogen to boron is in the range from two to four parts of nitrogen per part of boron, products having good magnetic properties can not be consistently produced even though the boron content of the melt is within the above stated critical range. Consequently, in accordance with this invention, the nitrogen content of the melt will be in the range from about 15 parts per million to about 95 parts per million.

The nitrogen requirement can be met in any convenient manner, but in preferred practice the metal in a vacuum furnace is provided with a 30-torr nitrogen atmosphere to which argon is added to bring the pressure up to one atmosphere for the pouring operation. The metal as poured contains about 30 ppm of nitrogen and in the neighborhood of 10 ppm of boron. The pressure of nitrogen required in the furnace chamber will depend in any given circumstance upon the ratio of the volume of the chamber to the weight of the melt.

Another discovery which I have made is that the proportions of sulfur and manganese in the metal during final annealing treatment are critical in terms of the magnetic properties of the final product strip or sheet material. Particularly, it is essential that there be at least 0.007 percent sulfur in solute form at that stage of processing. That requirement can be met if both the sulfur and the manganese contents of the silicon iron are quite low and in fact if there is no more than about 0.007 percent sulfur in the metal. The tendency for the manganese to tie up the sulfur is negligible in highly dilute systems in which the manganese content is of the order of about 0.002 to 0.006 percent and, consequently, it is not necessary in the practice of this invention to reduce the manganese content of the metal to a trace amount under any circumstances.

From the foregoing it will be understood that this invention has both method and article or product aspects. Thus, the several discoveries and new concepts set forth above expressed in terms of manipulative steps add up to a novel process and when expressed in compositional terms define a unique silicon-iron sheet product. The product is a cold-rolled sheet of final gauge thickness which by virtue of its boron, nitrogen, manganese and sulfur content can be converted to the oriented state in which it will have valuable magnetic properties but will not contain the boron which enabled the development of those properties through secondary recrystallization. The process of producing this new intermediate cold-rolled sheet is also new as is the overall process of producing the final desired sheet material from a silicon-iron melt.

Briefly described in its article aspect, this invention comprises a cold-rolled silicon-iron sheet product containing 2.2 to 4.5 percent silicon, between about 5 and 45 ppm boron, between about 15 and 95 ppm nitrogen with the nitrogen and boron being in the ratio range of 2 to 4 parts of nitrogen per part of boron, between about 0.007 and 0.06 percent sulfur, and between about 0.002 and 0.01 percent manganese, and the proportion of manganese to sulfur being such that the presence in the metal of at least 0.007 percent sulfur in solute form is assured during the final texture anneal.

Similarly described, the method comprises the steps of providing this intermediate sheet product and subjecting it to a final heat treatment to develop (110)[001] secondary recrystallization texture in it.

#### 5 DETAILED DESCRIPTION OF THE INVENTION

In the preferred practice of this invention, the amount of nitrogen in the metal will not exceed about 60 ppm so that any tendency for nitrogen-induced slivering and blistering can be avoided. This requirement is readily met by commercial steel-producing practices when usual precautions are taken to limit nitrogen pick-up. Consequently, it is preferable to add boron to the melt after it has been tapped into the ladle for teeming. The amounts to be added will be 10-20 ppm of the melt weight.

In carrying out the method of this invention, one will prepare a silicon-iron melt of required chemistry and use it to produce ingots which are hot rolled to intermediate thickness. When it is poured, the melt will contain from 2.2 to 4.5 percent silicon, from 0.003 to 0.06 percent sulfur, from 0.001 to 0.10 percent manganese and from about 5 to 45 parts per million boron, from about 15 to 95 parts per million nitrogen in the ratio range to boron between two and four parts to one, the remainder being iron and small incidental amounts of other elements including carbon, aluminum and oxygen. The resulting sheet is cold rolled to final gauge thickness and subjected to the final heat treatment for decarburization and development of the (110)[001] secondary recrystallization texture. Preferably, hot rolling will be carried out between 1,100° and 1,350°C and the hot-rolled sheet will be pickled and then may be heat treated suitably for several minutes at 900° to 1,000°C before cold rolling. Cold rolling may be in one stage or in two stages with an intermediate anneal. Also, the decarburization heat treatment at final gauge will be carried out at 800°C in hydrogen containing sufficient moisture to effect the removal of carbon. A heat treatment of 1 to 5 minutes is used for this purpose. In the final texture anneal, secondary grain growth to produce the desired texture is initiated at about 950°C when heating at 50°C per hour in pure nitrogen. Recrystallization should be completed by the time the temperature attains 1,000°C and a change of atmosphere to purified dry hydrogen can then be made. Heating can be continued to about 1,025°C for a low temperature anneal, or to higher temperatures such as 1,175°C for 50 more complete removal of residual sulfur, carbon and nitrogen.

In mill operations, the sulfur content of silicon-iron melts normally is substantially greater than the tolerable level in finished electrical steel sheet products. Accordingly, taking full advantage of the unique opportunity afforded by this invention for use of a lower sulfur content during the texture-developing stage of the final heat treatment, one will subject the melt to a desulfurization step. Preferably, this is accomplished in the ladle prior to teeming through the addition of lime and fluorospar to the ladle so that the sulfur content of the metal is reduced to a level nearer the limit specified for the ultimate sheet product.

65 The following illustrative, but not limiting, examples of my novel method as I have actually carried it out will further inform those skilled in the art of the nature and special utility of this invention:

## EXAMPLE I

A vacuum furnace was used to prepare a silicon-iron melt of the following composition:

|           |                      |
|-----------|----------------------|
| Silicon   | 3.25 per cent        |
| Sulfur    | 0.009 per cent       |
| Manganese | 0.002 per cent       |
| Carbon    | 0.024 per cent       |
| Boron     | 6 parts per million  |
| Aluminum  | 47 parts per million |
| Nitrogen  | 27 parts per million |
| Oxygen    | 18 parts per million |
| Iron      | Remainder            |

The furnace was charged with electrolytic iron and a carbon addition and the melt was held in the molten condition for as long as one hour to enable reduction of boron from the crucible. The ferrosilicon, ferrous sulfide and a final carbon addition were added and the melt was poured to produce an ingot ( $11 \times 5\frac{1}{2} \times 2\frac{1}{8}$  inches). The ingot was heated to  $1,325^{\circ}\text{C}$  for 45 minutes under a hydrogen atmosphere and then hot rolled to a sheet of about 0.085 inch thickness using eight passes without reheating. Pieces were cut from the hot-rolled sheet for reduction by cold rolling after pickling to remove hot-rolling scale and normalizing for 5 minutes at  $900^{\circ}\text{C}$  in hydrogen (dewpoint about  $0^{\circ}\text{F}$ ). The sheet was cold rolled without tension to 0.028 inch thickness and then normalized 3 minutes at  $900^{\circ}\text{C}$  in hydrogen (dewpoint about  $0^{\circ}\text{F}$ ) and again cold rolled (but with tension) to 0.011 inch thickness. Test strips 3 cm by 30.5 cm in size were sheared in the rolling direction from this strip, sufficient to form an Epstein test pack. The strips were decarburized by heating for three minutes at  $800^{\circ}\text{C}$  in wet hydrogen ( $+70^{\circ}\text{F}$  dewpoint). They were then annealed as a pack by heating at  $50^{\circ}\text{C}$  per hour in purified nitrogen to  $975^{\circ}\text{C}$ , then in purified hydrogen at the same rate of heating to  $1,024^{\circ}\text{C}$ , holding 3 hours at this temperature followed by cooling at  $50^{\circ}\text{C}$  per hour in hydrogen to  $600^{\circ}\text{C}$  to room temperature, cooling was accomplished by withdrawal of the retort to the cooling zone of the furnace. Magnetic test results are given below. When this same pack was reannealed, heating in hydrogen to  $1,175^{\circ}\text{C}$ , magnetic properties were only slightly improved. Thus, a material requiring only a relatively low temperature anneal to develop good magnetic quality is demonstrated.

## Magnetic Properties

| Heat Treatment  | Thickness (mils) | A.C. Loss              |         |                |
|-----------------|------------------|------------------------|---------|----------------|
|                 |                  | at 60 Hertz<br>15,000B | 16,300B | $\mu\text{OH}$ |
| 1025°C anneal   | 10.7             | 0.537                  | 0.647   | 1856           |
| 1175°C reanneal | 10.7             | 0.529                  | 0.644   | 1862           |

|           |                      |
|-----------|----------------------|
| Silicon   | 3.28 per cent        |
| Sulfur    | 0.009 per cent       |
| Manganese | 0.002 per cent       |
| Carbon    | 0.024 per cent       |
| Boron     | 6 parts per million  |
| Aluminum  | 47 parts per million |
| Nitrogen  | 27 parts per million |
| Oxygen    | 18 parts per million |
| Iron      | Remainder            |

Again, as in Example I, the resulting ingot was hot rolled and otherwise processed as described therein with the result that a product was obtained corresponding to that of Example I having permeability of 1,865 gausses per oersted (in a 10-oersted field), and losses of 0.553 and 0.665 watts per pound at 15,000 and 16,300 gausses, respectively, following anneal at  $1,025^{\circ}\text{C}$ .

## EXAMPLE III

In the preparation of the melt for this example, a change was made from the method of Example I. The melt was held in the crucible in molten condition for only a few minutes in order to limit the reduction of boron from the crucible. A boron addition as a 19 percent grade ferroboron was made to the melt after the ferrosilicon, ferrous sulfide and final carbon additions had been made. The resulting composition as determined by analysis was as follows:

|           |                      |
|-----------|----------------------|
| Silicon   | 3.25 per cent        |
| Sulfur    | 0.008 per cent       |
| Manganese | 0.003 per cent       |
| Carbon    | 0.02 per cent        |
| Boron     | 12 parts per million |
| Nitrogen  | 37 parts per million |
| Oxygen    | 30 parts per million |
| Iron      | Remainder            |

The procedure for hot rolling was modified from that of Example I in that the rolled billet at  $1\frac{1}{2}$  inch thickness was cooled to room temperature and divided into several pieces. These were reheated to one of several temperatures, used to continue hot rolling to 0.08 inch thick sheet. For the material of this example, a  $1,300^{\circ}\text{C}$  reheat temperature was used. The total number of passes and the reduction for each pass were unchanged.

Cold rolling was carried out in two stages with an intermediate thickness of 0.05 inch. The intermediate heat treatment was at  $900^{\circ}\text{C}$  for 3 minutes in dry hydrogen as before. After cold rolling to a final thickness of 0.011 inch, Epstein strips were cut, decarburized at  $800^{\circ}\text{C}$  in hydrogen of room temperature dewpoint, and annealed as in Example I. Magnetic test values after annealing at  $1,025^{\circ}\text{C}$ , and again at  $1,175^{\circ}\text{C}$  were as follows:

| Heat Treatment | Thickness (inches) | A.C. Loss at 60 Hertz |         |                |
|----------------|--------------------|-----------------------|---------|----------------|
|                |                    | 15,000B               | 16,000B | $\mu\text{OH}$ |
| 1025°C anneal  | 0.0107             | 0.547                 | 0.656   | 1856           |
| 1175°C anneal  | 0.0108             | 0.503                 | 0.600   | 1867           |

## EXAMPLE II

Following the procedure described in Example I, the silicon-iron melt of the following composition was prepared:

## EXAMPLE IV

A melt of the following composition was prepared as described in Example III:

|           |                      |
|-----------|----------------------|
| Silicon   | 3.25 per cent        |
| Sulfur    | 0.008 per cent       |
| Manganese | 0.008 per cent       |
| Carbon    | 0.022 per cent       |
| Boron     | 12 parts per million |
| Nitrogen  | 22 parts per million |
| Oxygen    | 37 parts per million |
| Iron      | Remainder            |

An ingot of the size already described was poured and hot and cold rolled with intermediate heat treatments as described in Example I. The resulting 11-mil strip when prepared as an Epstein pack and annealed as in

5 Example I developed the following magnetic properties:

| Heat Treatment  | Thickness (mils) | A.C. Loss at 60 Hertz |                       |                      |
|-----------------|------------------|-----------------------|-----------------------|----------------------|
|                 |                  | 15,000 gs. (watts/lb) | 16,300 gs. (watts/lb) | $\mu$ 10H (watts/lb) |
| 1025°C anneal   | 10.7             | 1.075                 | 1.187                 | 1463                 |
| 1175°C reanneal | 10.7             | 1.143                 | 1.256                 | 1441                 |

The resulting magnetic properties after processing as set forth in Example III, except that a reheat temperature of 1,150°C was used in hot rolling, were:

| Heat Treatment  | Thickness (inches) | A.C. Loss at 60 Hertz |                       |           |
|-----------------|--------------------|-----------------------|-----------------------|-----------|
|                 |                    | 15,000 gs. (watts/lb) | 16,300 gs. (watts/lb) | $\mu$ 10H |
| 1025°C anneal   | 0.0107             | 0.508                 | 0.611                 | 1876      |
| 1175°C reanneal | 0.0108             | 0.497                 | 0.589                 | 1882      |

### EXAMPLE V

A melt of the following composition was prepared in accordance with the procedure set forth in Example III:

|           |                      |
|-----------|----------------------|
| Silicon   | 3.3 per cent         |
| Sulfur    | 0.006 per cent       |
| Manganese | 0.005 per cent       |
| Carbon    | 0.002 per cent       |
| Boron     | 50 parts per million |
| Aluminum  | 30 parts per million |
| Nitrogen  | 24 parts per million |
| Oxygen    | 24 parts per million |
| Iron      | Remainder            |

The resulting ingot was hot and cold rolled and otherwise processed as described in Example III. The resulting sheet product had magnetic properties after annealing of:

| Heat Treatment  | Thickness (mils) | A.C. Loss at 60 Hertz |                       |           |
|-----------------|------------------|-----------------------|-----------------------|-----------|
|                 |                  | 15,000 gs. (watts/lb) | 16,300 gs. (watts/lb) | $\mu$ 10H |
| 1025°C anneal   | 10.7             | 1.226                 | 1.379                 | 1465      |
| 1175°C reanneal | 10.7             | 1.149                 | 1.266                 | 1443      |

### EXAMPLE VI

In an operation similar to that of Example III wherein a minimum opportunity was provided for the reduction of boron from the crucible, and no boron addition was made to the melt, a melt of the following composition was prepared:

|           |                      |
|-----------|----------------------|
| Silicon   | 3.5 per cent         |
| Sulfur    | 0.008 per cent       |
| Manganese | 0.002 per cent       |
| Carbon    | 0.029 per cent       |
| Boron     | 2 parts per million  |
| Aluminum  | 27 parts per million |
| Nitrogen  | 22 parts per million |
| Oxygen    | 19 parts per million |
| Iron      | Remainder            |

25 A full-scale mill heat of 159,000 pounds of silicon-iron was prepared using metal from a basic oxygen furnace. The melt was desulfurized (sulfur reduced from 0.020 to 0.007 percent) as it was tapped and poured into a ladle containing 2,000 pounds of burned lime and 600 pounds of fluor spar. Iron sulfide was then 30 added to bring the sulfur content from 0.007 to 0.009 percent, and 5 pounds of 19 percent grade ferroboron were added to the ladle for purposes of the experiment. The analysis of the metal in the ladle was then as follows:

|           |           |            |         |
|-----------|-----------|------------|---------|
| Silicon   | 3.20%     | Aluminum   | 0.005%  |
| Manganese | 0.030%    | Phosphorus | 0.006%  |
| Carbon    | 0.033%    | Titanium   | 0.005%  |
| Nickel    | 0.094%    | Nitrogen   | 0.0033% |
| Copper    | 0.24%     | Oxygen     | 0.0052% |
| Tin       | 0.021%    | Sulfur     | 0.009%  |
| Chromium  | 0.043%    | Boron      | 0.0008% |
| Iron      | Remainder |            |         |

45 Ingots cast from the metal were hot rolled from 2,450°F to 90 mils thickness and then pickled, as described in Example I, heat treated for 5 minutes at 900°C, cold rolled to 0.028 inch thickness, heat treated 3 minutes at 900°C, and cold rolled to a final gauge of 0.011 inch. Test strips were sheared in the rolling direction to form an Epstein pack and were decarburized by a 3-minute heat treatment in hydrogen of 70°F dew point. The strips were then annealed by heating at a rate of 50°C per hour in nitrogen from 800°C to 950°C, then at the same rate in dry hydrogen to 1,025°C. After 50 holding 3 hours at this temperature, the strips were cooled at 50°C per hour in hydrogen to 600°C at which temperature the annealing retort was withdrawn to the cooling chamber. The measured magnetic properties 55 were:

| Heat Treatment | Thickness (mils) | A.C. Loss at 60 Hertz   |                         |           |
|----------------|------------------|-------------------------|-------------------------|-----------|
|                |                  | 15,000 gauss (watts/lb) | 16,300 gauss (watts/lb) | $\mu$ 10H |
| 65             | 10.4             | 0.590                   | 0.739                   | 1805      |

## EXAMPLE VIII

In another operation similar to that of Example III, a melt of the following composition was prepared:

|           |        |           |
|-----------|--------|-----------|
| Silicon   | 3.28   | per cent  |
| Manganese | 0.001  | per cent  |
| Sulfur    | 0.005  | per cent  |
| Carbon    | 0.018  | per cent  |
| Aluminum  | 0.004  | per cent  |
| Boron     | 0.0007 | per cent  |
| Nitrogen  | 0.0019 | per cent  |
| Oxygen    | 0.0026 | per cent  |
| Iron      |        | Remainder |

An ingot was poured and processed through hot and cold rolling stages and heat treatments as described in Example I and test strips of the resulting 11-mil material were used to provide an Epstein pack. This pack was heated at 50°C per hour in purified nitrogen to 975°C where it was held for 3 hours and then cooled at the rate of 50°C per hour at 600°C, whereupon it was placed in a cooling zone of the furnace until the pack reached room temperature. The product proved to have good properties when tested as described above, permeability being 1,898 gausses per oersted (in a 10-  
0ersted field).

A series of experiments was performed for purposes of determining the effects of various boron and nitrogen ratios on the development of secondary recrystallization during the final anneal. Thus, a total of six separate heats were prepared, all of the following basic composition:

|         |       |           |
|---------|-------|-----------|
| Silicon | 3.25  | per cent  |
| Sulfur  | 0.008 | per cent  |
| Carbon  | 0.025 | per cent  |
| Iron    |       | Remainder |

To four of the heats, ferroboron was added to provide a nominal composition of 50 parts per million boron, while the boron content of the other two was nominally established at 50 and 75 parts per million. The nitrogen content ranged in these heats from 40 to 145 parts per million.

## EXAMPLE IX

The partial pressure of nitrogen in the furnace was maintained at 30 mm, and the metal was poured from the ladle following the ferroboron addition. The resulting ingot was hot and cold rolled and heat treated as described in Example III. Analysis of the cold-rolled strip indicated the boron content to be 30 ppm and the nitrogen content to be 41 ppm. Magnetic properties of the cold-rolled strip product are set out in Table A below together with those of the following examples.

## EXAMPLE X

Following the procedure of Example IX except that the nitrogen partial pressure in the furnace was 60 mm, a cold-rolled product was obtained which proved on analysis to contain 30 ppm boron and 53 ppm nitrogen.

## EXAMPLE XI

Following the procedure of Examples IX and X, but still further increasing the partial pressure of nitrogen in the furnace to 100 mm, resulted in a cold-rolled product which was similarly found to contain 32 ppm boron and 78 ppm nitrogen.

## EXAMPLE XII

Again, the procedure of Example IX was followed with the exception that the partial pressure of nitrogen in the furnace was 400 mm. The cold-rolled product contained 34 ppm boron and 145 ppm nitrogen.

## EXAMPLE XIII

Following the Example IX procedure, but maintaining 200 mm nitrogen partial pressure in the furnace and adding still more ferroboron to the ladle, resulted in a cold-rolled product containing 59 ppm boron and 68 ppm nitrogen.

## EXAMPLE XIV

A cold-rolled strip product which contained on analysis 44 ppm boron and 93 ppm nitrogen was made generally in the manner described in Example IX through the addition to the ladle of ferroboron in amount equivalent to 50 ppm boron and by maintaining the nitrogen partial pressure in the melting furnace at 200 mm.

TABLE A

| Example | Thickness (in.) | A.C. Loss |       |           |
|---------|-----------------|-----------|-------|-----------|
|         |                 | 15kB      | 17kB  | $\mu$ 10H |
| IX      | .0108           | 1.271     | —     | 1421      |
| X       | .0108           | .687      | 1.014 | 1669      |
| XI      | .0107           | .518      | .676  | 1894      |
| XII     | .0107           | .930      | 1.255 | 1551      |
| XIII    | .0107           | 1.139     | —     | 1413      |
| XIV     | .0107           | .539      | .712  | 1842      |

Whenever in this specification and in the appended claims reference is made to amounts, rates, percentages, or proportions, the weight basis is intended unless otherwise expressly stated.

As used herein and in the appended claims, the term "ingot" means and refers to a body made by solidifying by any casting method a molten steel made by any suitable steel-making method, and this includes a slab-like ingot obtained by a continuous casting method.

What I claim as new and desire to secure by Letters Patent of the United States is:

1. The method of producing grain-oriented silicon-iron sheet which comprises the steps of providing a silicon-iron melt containing 2.2 to 4.5 percent silicon and lesser amounts of sulfur and manganese, incidental amounts of other elements including carbon, aluminum and oxygen, and balance iron, adding a source of boron to the melt, casting the melt and hot-rolling the resulting billet to form an elongated sheet-like body, cold-rolling the hot-rolled sheet-like body to provide a sheet of final gauge thickness containing from 5 to 45 parts per million boron and from about 15 to 95 ppm nitrogen and the proportions of nitrogen and boron being in the ratio range of two to four parts of nitrogen to one part of boron, from 0.007 to 0.06 percent sulfur and from 0.002 to 0.1 percent manganese and the proportions of the sulfur and manganese being such as to result in a minimum of about 0.007 percent sulfur in solute form during final annealing treatment, and subjecting the said cold-rolled sheet to a final heat treatment to decarburize it and to develop (110) [001] secondary recrystallization texture in it.
2. The method of claim 1 in which the amount of boron in the cold-rolled sheet is between about 5 and about 20 ppm.

3. The method of claim 1 in which the cold-rolled sheet contains 12 to 20 parts per million of boron, 3.25 percent silicon, 0.008 percent manganese, 0.008 percent sulfur, and 37 ppm oxygen, iron constituting the remainder, and in which the final anneal consists of heating in an atmosphere consisting primarily of nitrogen until secondary recrystallization is completed, and then completing the annealing treatment in pure hydrogen.

4. The method of claim 1 which includes the preliminary step of reducing the sulfur and manganese contents of the melt to less than about 0.01 percent.

5. The method of claim 1 which includes the preliminary step of adding a desulfurizing agent to the melt and thereby reducing the sulfur content of the melt from about 0.020 to 0.025 percent to about 0.005 to 0.010 percent.

6. The method of claim 1 in which the melt contains about 0.03 percent manganese and about 0.020 to 0.025 percent sulfur, and which includes a desulfurizing step comprising the addition of lime and fluorospar to the melt to reduce the sulfur content thereof to less than about 0.010 percent.

7. The method of claim 1 in which the cold-rolled sheet contains about 30 parts per million boron and about 80 parts per million nitrogen.

8. The method of claim 1 in which the cold-rolled sheet contains about 45 ppm boron and about 95 ppm

nitrogen.

9. The method of producing grain-oriented silicon-iron sheet which comprises the steps of providing a cold-rolled sheet of the thickness of the desired final product and containing 2.2 to 4.5 percent silicon, from about 5 to about 45 ppm boron, about 15 to 95 ppm nitrogen and the proportions of nitrogen and boron being in the ratio range of two to four parts of nitrogen to one part of boron, from about 0.007 to 0.06 percent sulfur, and from 0.002 to 0.1 percent manganese and the proportion of sulfur and manganese being such as to result in a minimum of about 0.007 percent sulfur in solute form during the final annealing treatment, and subjecting the said cold-rolled sheet to a final heat treatment to decarburize it and to develop (110)[001] secondary recrystallization texture in it.

10. A cold-rolled silicon-iron sheet product containing 2.2 to 4.5 percent silicon, between about 5 and 45 parts per million boron, between about 15 and 95 ppm nitrogen, the amounts of nitrogen and boron being in the ratio range of two to four parts of nitrogen per part of boron, between about 0.007 and 0.06 percent sulfur, and between about 0.002 and 0.1 percent manganese, the proportion of sulfur to manganese being such as to result in a minimum of about 0.007 percent sulfur in solute form when the sheet is heated to about 950°C during texture-developing heat treatment.

\* \* \* \* \*